

## UNITED STATES PATENT OFFICE

2,058,418

## DYEING PROCESS

Miles A. Dahlen, Stanley R. Detrick, Robert E. Etzelmiller, and Frithjof Zwigmeyer, Wilmington, Del., assignors to E. I. du Pont de Nemours & Company, Wilmington, Del., a corporation of Delaware

No Drawing. Application April 2, 1935,  
Serial No. 14,270

18 Claims.

(Cl. 8—6)

This invention relates to new dyeing and printing processes and more particularly refers to improved processes for dyeing and printing cotton and related textile materials by means of mixtures of ice color coupling components and diazoimino compounds to be more fully described hereafter.

Certain classes of diazoimino compounds which are well adapted for use in the dyeing and printing of textile materials have been described in the prior art. The stabilizing components of these compounds are all characterized in that they are hydrocarbons containing an amino or imino group and one or more carboxylic or sulfonic acid groups. With the exception of the aforementioned substituents, however, the stabilizing components are composed entirely of carbon and hydrogen. For a more detailed description of compounds of this type reference may be made to U. S. Patents 1,882,560, 1,882,561, 1,882,562 and 1,982,681.

Since the coupling of diazotized arylamines and tetrazotized arylene diamines with various components is profoundly affected by the structure of such components it is exceedingly important that great care be exercised in selecting coupling components. This is true to an even greater extent in the production of diazoimino compounds because of additional characteristics which these compounds must possess. For example, a satisfactory diazoimino compound must couple in such manner that the resulting product is stable in neutral or alkaline solution. Moreover, the product must be readily soluble. Of equal importance is the ability of these compounds to hydrolyze readily and completely in order that the diazo base might be satisfactorily regenerated. It is obvious from a consideration of these factors that the structure of the stabilizing component is of utmost importance and that the presence thereon of certain substituents, as well as the position of these substituents, produces a far reaching effect upon the characteristics of the resulting compound.

It is an object of this invention to devise an entirely new process for dyeing and printing textile materials. A further object is to produce a color imparting medium which may exist in the form of dry powders, aqueous pastes, aqueous solutions, or other types of solutions. A still further object is to produce a dyeing and printing medium which contains a class of diazoimino compounds which is entirely unrelated to any heretofore used. A still further object is to utilize a unique and heretofore unknown class of

diazoimino compounds in the production of ice colors on cotton fibers. Additional objects will become apparent from a consideration of the following description and claims.

These objects are attained according to the herein described invention wherein dyeing and printing compositions are made which contain the customary coupling components, assistants and the like, in addition to diazoimino compounds produced by coupling a diazotized aromatic amine or tetrazotized aromatic diamine with a heterocyclic compound having an imino-containing radical substituted thereon. In a more restricted sense this invention is concerned with dyeing and printing compositions containing an ice color coupling component and a water and alkali soluble diazoimino compound produced by coupling a diazotized aromatic amine, capable of use in the production of ice colors, with a heterocyclic compound having an imino-containing radical substituted thereon through the imino group of which coupling takes place, and furthermore containing one or more water-solubilizing groups. This invention pertains, in its preferred embodiment, to dyeing and printing compositions containing approximately molecular equivalent quantities of an ice color coupling component, preferably arylamides of 2-3-hydroxy-naphthoic acid or acyl-acet-arylates, and diazoimino compounds produced by coupling diazotized aromatic amines, capable of use in the production of ice colors, with furfuryl-amino-acetic acid or tetra-hydro-furfuryl-amino-acetic acid.

The invention may be more readily understood by a consideration of the following illustrative examples in which the quantities are stated in parts by weight:

## Example 1

40

330 parts of the dry diazoimino compound of the following formula:



obtained by the action of diazotized 4-chloro-2-amino-toluene on furfuryl-amino-acetic acid, were ground with 280 parts of the ortho-toluidide

55

of 2-3-hydroxy-naphthoic acid producing a yellow powder.

A printing paste of the following composition was prepared:

|                                 | Parts |
|---------------------------------|-------|
| 5 The above mixture             | 4.0   |
| Cellosolve                      | 4.0   |
| Sodium hydroxide solution (35%) | 2.0   |
| Sulfonated castor oil           | 1.0   |
| 10 Water (warmed to 140° F.)    | 29.0  |
| Starch tragacanth thickener     | 60.0  |
|                                 | 100.0 |

15 and printed from an engraved roll onto cotton piece goods. The printed material was dried thoroughly and then aged for 2½ minutes in the vapors arising from a boiling solution of 4 parts of acetic acid (56%) and 1 part of formic acid (85%) in 15 parts of water. The prints were rinsed, soaped, again rinsed, and then dried. Bright red dyeings of good fastness properties were obtained, due to the formation of the dye of the formula:



*Example 2*

35 334 parts of the dry diazoimino compound of the following formula:



obtained by the action of diazotized 4-chloro-2-amino-toluene with tetra-hydro-furfuryl-amino-acetic acid, was mixed with 400 parts of diacetoxycetyl-ortho-tolidine. Cotton piece goods were 50 printed with a paste prepared from this composition by the process described in Example 1. The printed pattern was developed as a bright yellow of moderate fastness properties, due to the production of the dye of the formula:



*Example 3*

350 parts of the water soluble diazoimino compound of the following structural formula:



produced by the action of diazotized 4-chloro-2-amino-anisole on furfuryl-amino-acetic acid was mixed with 300 parts of the ortho-aniside of 2-3-hydroxy-naphthoic acid. Cotton piece goods were printed with a paste prepared from this composition by the procedure similar to that described in Example 1. After color development and soaping of the prints, the pattern was developed as a brilliant bluish red due to the formation of the color of the probable formula:



*Example 4*

20

350 parts of the water soluble diazoimino compound of the following formula:



obtained by the action of diazotized 4-chloro-2-amino-anisole on tetra-hydro-furfuryl-amino-acetic acid, and 225 parts of aceto-acetyl-p-phenetidine were stirred with 600 parts of ethyl alcohol, 300 parts of sodium hydroxide solution of 30% strength were added, followed by 1400 parts of water. The mass was stirred until complete solution was obtained, then filtered.

A printing paste of the following composition was prepared:

|                             | Parts |
|-----------------------------|-------|
| The above solution          | 20    |
| Water                       | 20    |
| Starch tragacanth thickener | 60    |

Cotton goods were printed and aged by the procedure given in Example 1. Bright yellow dyeings of very good fastness to light were obtained, due to the formation of the dye of the formula:



*Example 5*

65

335 parts of the dry diazoimino compound of the following formula:



obtained by the action of diazotized 4-chloro-2-amino-anisole on tetra-hydro-furfuryl-amino-acetic acid, were ground with 240 parts of aceto-acetyl-p-phenetidine producing a gray powder.

5 12 parts of this mixture were dissolved in 40 parts of sodium hydroxide solution (35%) and 950 parts of water. Cotton piece goods were padded in this solution, then passed through squeeze rollers and dried. The padded goods were aged under the 10 same conditions given in Example 1, rinsed, soaped, rinsed and dried. Bright yellow dyeings of good fastness to light were obtained. The color was identical with that produced according to Example 4.

15 The following table lists a number of other representative dyeing and printing compositions, suitable for the coloring of textile fabrics as illustrated in the above examples:

| No. | Base                                             | Stabilizer                                                                         | Coupling component                                       | Shade produced | 20 |
|-----|--------------------------------------------------|------------------------------------------------------------------------------------|----------------------------------------------------------|----------------|----|
| 1   | 4-chloro-2-aminotoluene                          | Tetra-hydro-furfuryl-amino-acetic acid                                             | 2-hydroxy-3-naphthoyl-o-toluidine                        | Red.           |    |
| 2   | do                                               | do                                                                                 | 2-hydroxy-3-naphthoyl-o-phenetidine                      | Scarlet.       |    |
| 25  | do                                               | do                                                                                 | Sodium compound of 2-hydroxy-3-naphthoyl-m-xylidine      | Red.           | 25 |
| 4   | 4-chloro-2-amino-anisole                         | do                                                                                 | 2-hydroxy-3-naphthoyl-o-anisidine                        | Do.            |    |
| 5   | 4-nitro-2-amino-anisole                          | do                                                                                 | 2-hydroxy-3-naphthoyl-3'-nitro-anisidine                 | Bluish-red.    |    |
| 6   | Dianisidine                                      | do                                                                                 | Sodium compound of 2-hydroxy-3-naphthoyl-aniline         | Blue.          |    |
| 7   | 4-furyl-amino-2,5-diethoxy-aniline               | do                                                                                 | 2-hydroxy-3-naphthoyl-aniline                            | Do.            |    |
| 8   | 4-carbomethoxy-amino-2,5-dimethoxy-aniline       | do                                                                                 | 2-hydroxy-3-naphthoyl-anisidine                          | Do.            | 30 |
| 9   | 3-chloro-aniline                                 | do                                                                                 | Sodium compound of 2-hydroxy-3-naphthoyl-o-naphthylamine | Red.           |    |
| 10  | 5-nitro-2-amino-anisole                          | do                                                                                 | Diacet-o-acetyl-o-toluidine                              | Bordeaux.      |    |
| 11  | 2,5-dichloro-aniline                             | 1-(furfuryl-amino)-ethane-2-sulfonic acid                                          | Sodium compound of 2-hydroxy-3-naphthoyl-o-toluidine     | Yellow.        |    |
| 12  | 4-furyl-amino-2,5-dimethoxy-aniline              | do                                                                                 | Sodium compound of 2-hydroxy-3-naphthoyl-o-toluidine     | Red-blue.      |    |
| 35  | 13 4-ethoxy-4'-amino-2'-5'-dimethoxy-azo-benzene | do                                                                                 | Sodium compound of 2-hydroxy-3-naphthoyl-o-toluidine     | Black.         | 35 |
| 14  | 4-chloro-2-amino-anisole                         | do                                                                                 | Sodium compound of 2-hydroxy-3-naphthoyl-o-naphthylamine | Yellow.        |    |
| 15  | 4-benzoyl-amino-2,5-diethoxy-aniline             | do                                                                                 | Aceto-acetyl-p-phenetidine                               | Green.         |    |
| 16  | 4-chloro-2-amino-toluene                         | do                                                                                 | 2-hydroxy-anthracene-3-carboxylic acid-o-toluidide       | Red.           |    |
| 40  | 17 do                                            | do                                                                                 | Sodium compound of 2-hydroxy-3-naphthoyl-o-toluidine     | Yellow.        | 40 |
| 18  | Aniline                                          | do                                                                                 | Diacet-o-acetyl-o-toluidine-sulfone                      | Do.            |    |
| 19  | 4'-ethoxy-4-amino-diphenyl-amine                 | do                                                                                 | 2-hydroxy-3-naphthoyl-aniline                            | Blue.          |    |
| 20  | Dianisidine                                      | do                                                                                 | do                                                       | Do.            |    |
| 21  | do                                               | Furfuryl-amino-acetic acid                                                         | 2-hydroxy-3-naphthoyl-o-toluidine                        | Do.            |    |
| 22  | 3-benzoyl-amino-4-methoxy-aniline                | do                                                                                 | 2-hydroxy-3-naphthoyl-aniline                            | Bordeaux.      |    |
| 23  | 4-carbomethoxy-amino-2,5-diethoxy-aniline        | do                                                                                 | 2-hydroxy-3-naphthoyl-o-toluidine                        | Blue.          |    |
| 45  | 24 4-benzoyl-amino-2-methoxy-5-methyl-aniline    | do                                                                                 | Sodium compound of 2-hydroxy-3-naphthoyl-aniline         | Violet.        | 45 |
| 25  | 4-chloro-2-amino-toluene                         | A mixture of furfuryl-amino-acetic acid and tetra-hydro-furfuryl-amino-acetic acid | Sodium compound of 2-hydroxy-3-naphthoyl-o-toluidine     | Red.           |    |
| 26  | do                                               | β-hydroxy-ethyl-furfuryl-amine                                                     | Sodium compound of 2-hydroxy-3-naphthoyl-o-phenetidine   | Scarlet.       |    |
| 50  | 27 do                                            | α-pyridyl-amino-acetic acid                                                        | Sodium compound of 2-hydroxy-3-naphthoyl-o-phenetidine   | Do.            | 50 |
| 28  | 4-chloro-2-amino-anisole                         | A mixture of furfuryl-amino-acetic acid and tetra-hydro-furfuryl-amino-acetic acid | p-chlor-anilide of 2-hydroxy-carbazole-3-carboxylic acid | Brown.         |    |
| 29  | 4-benzoyl-amino-2,5-diethoxy-aniline             | do                                                                                 | o-toluidide of 2-hydroxy-anthracene-3-carboxylic acid    | Green.         |    |

55 It is to be understood that the aforementioned examples are illustrative merely of a relative few of the many modifications of the present invention. It is contemplated that the individual components, the proportions thereof, the conditions of reaction and related features thereof may be varied widely without departing from the scope of this invention.

In place of the diazoimino compounds referred 65 to supra it is to be understood that other diazoimino compounds which contain as a stabilizing component a heterocyclic radical having substituted thereon an imino-containing radical and one or more water-solubilizing groups may be used. Primary arylamines and arylene diamines which are suitable for use in the production of ice colors may be used in manufacturing these diazoimino compounds. In this connection it may be stated that amines of the benzene, di-

ride, 3-amino-carbazole, alpha-amino-anthraquinone, 2,5-diethoxy-aniline, 5-methyl-2-methoxy-aniline, 5-chloro-2-amino-anisole and 4-chloro-4'-amino-2',5'-diethoxy-azobenzene.

As in the case of the arylamines, the stabilizing components may also be varied within a considerable range in accordance with the present invention. These stabilizing components are quite unrelated to any heretofore known or used in that they are not hydrocarbon derivatives but are heterocyclic compounds containing one or more hetero atoms and having an imino-containing radical substituted thereon. Coupling takes place through the imino group of the aforementioned radical. It is contemplated that additional groups 70 may be substituted upon the heterocyclic nucleus and/or upon the imino-containing radical previously referred to. Where additional substituents are added to the stabilizing component they should not be of such character, or substituted 75

on the component in such manner, that they interfere or prevent this coupling from taking place in the described manner. In order that the resulting diazoimino compounds may be soluble in water and/or alkali it is advisable to substitute one or more water-solubilizing groups upon the stabilizing component selected. These water-solubilizing groups are, for instance, carboxyl, sulfonic acid, hydroxyl, sulfonic acid, sulfato, and the like. The number and character of water-solubilizing groups which are desirable will depend to a great extent upon the diazo base selected and the purposes for which the resulting compounds are to be used. In general, the carboxylic acid and sulfonic acid groups are preferred. It is to be understood, however, that one or more of the additional solubilizing groups referred to or groups suggested thereby may be used in place of or in addition to the carboxylic and/or sulfonic acid group. A few representative stabilizing compounds selected in accordance with the above instructions are: Furfuryl-sorbitylamine, tetra-hydro-furfuryl-sorbityl-amine, 4-methylamino-2-furoic acid, 3-methylamino-25 benzopyrane-ar.-sulfonic acid, dioxanyl-amino-acetic acid, 3-(1'-methyl-morpholino)-glycine,  $\beta$ -thienyl-taurine,  $\alpha$ -thienyl-glucamine, (1:4-dimethyl-piperazino)-methyl-glycine, p-sulfo-phenyl-furfuryl-amine, p-hydroxy-cyclohexyl-tetra-30 hydro-furfuryl-amine, di-furfuryl-amino-4,4'-dicarboxylic acid and  $\beta$ -sulfato-ethyl-tetra-hydro-furfuryl-amine.

Many of the diazoimino compounds produced in accordance with the present invention may 35 be represented by the following general formula:



40 wherein aryl represents an aryl nucleus adapted for use as a component of an ice color, R<sub>1</sub> represents an alkyl, carbo-cyclyl, carbo-cyclyl-alkyl, hetero-cyclyl, or hetero-cyclyl-alkyl radical, R<sub>2</sub> represents a hetero-cyclyl or hetero-cyclyl-alkyl radical, and R<sub>1</sub> and/or R<sub>2</sub> contains one or more water-solubilizing groups.

45 Diazoimino compounds referred to herein which are of optimum value over a wide range of conditions and uses may be represented, for the most 50 part, by the following general formula:



55 wherein R represents the residue of a diazotized amine of the benzene or naphthalene series, free from water-solubilizing groups, and Z represents a furane derivative having an imino-containing radical substituted thereon, said furane derivative containing at least one water-solubilizing group.

60 Coupling components which are particularly adapted for use herein are those referred to by one familiar with the art as ice color coupling components. Among these components mention may be made of the following:

65 (1) Arylamides of hydroxy-aryl-carboxylic acids, such as the arylides of 2-3-hydroxy-naphthoic acids, 2-hydroxy-carbazole-3-carboxylic acid, 7-hydroxy-alpha-naphtho-carbazole-6-carboxylic acid, hydroxy-indole-carboxylic acids, hydroxy-diphenylamine-carboxylic acids, hydroxy-phenanthrene-carboxylic acids, etc. The arylamides may be produced from the usual primary arylamines free from water solubilizing groups, such as aniline, the halogenated anilines, toluidines, substituted toluidines, amino-phenol-ethers

and substitution products, naphthylamines and their substitution products, etc.

(2) Acyl-acetyl derivatives of arylamines, such as aceto-acetyl, benzoyl-acetyl, and terephthaloyl-bis-acetyl derivatives of primary arylamines and diamines free from water-solubilizing groups. 5

(3) Naphthols such as alpha- and beta-naphthol.

(4) Acyl-naphthols such as 4-benzoyl-1-naphthol and 4-acetyl-1-naphthol. 10

(5) Aryl-alkyl-pyrazolones.

(6) Dihydroxy-quinolines.

In general, it may be stated that the arylides of 15 2-3-hydroxy-naphthoic acid and acyl-acetyl derivatives of arylamines are preferred for use herein. It is to be understood that the invention is not restricted thereto, however, since the other ice color coupling components referred to supra, and the numerous additional components suggested thereby, are also capable of use herein. 20

In producing the dyeing and printing compositions described one or more of the diazoimino compounds coming within the scope of this invention may be mixed with one or more of the ice color coupling components referred to. Ordinarily it is advisable to select a single diazoimino compound and a single coupling component, the particular product selected depending to a large extent upon the color which is desired and the process whereby it is to be produced. For certain 30 purposes it is sometimes helpful to select a mixture of diazoimino compounds and/or coupling components, and the present invention is understood to be susceptible to such modification. The proportion of diazoimino compound and coupling 35 component present in the mixture may be varied within considerable range, although it is advisable that they be present in approximately molecular equivalent quantities. The customary dyeing and printing assistants may be incorporated in the 40 mixture when desired. When the coupling components are arylamides of hydroxy-naphthoic acids or related compounds they may be used in the form of the free acids or as salts, preferably in the form of alkali metal salts. It is clear from 45 a consideration of the preceding instructions that the resulting mixtures may be in the form of dry powders, aqueous pastes, aqueous solutions or other types of solutions, and when dyeing and printing compositions are mentioned in the present specification and claims it is understood that they embrace the aforementioned types of mixtures.

When solutions or aqueous pastes of the diazoimino compounds are produced it is advisable to make them sufficiently alkaline to prevent 55 hydrolysis of the diazoimino compounds to the parent diazo salts. It is frequently advantageous to utilize organic solvents in the preparation of these dyeing and printing solutions. Organic solvents of particular value in this connection are 60 water-miscible solvents, such as methanol, ethyl alcohol, ethylene glycol, alkyl ethers of ethylene glycol, diethylene glycol, and the like.

In imparting colors to textile fibers it is contemplated that the various procedures known to 65 the art may be followed. For example, when textile fibers are printed with pastes containing the described compositions color development may be effected by subjecting the prints to the action of steam and a mild volatile acid, such as acetic 70 and/or formic acids. Moreover, the prints may be developed by immersion in a boiling saturated salt solution which contains a weak acid, such as acetic, phthalic, oxalic, citric, and the like acids. It is also contemplated that materials may be in- 75

corporated in the printing pastes which are non-acidic in nature but which produce acids upon heating. A few of the many materials which come within this category are sodium chloracetate, diethanolamine sulfate and formamide. In the development of these prints and dyes the use of elevated temperatures is advantageous. As is clear from a consideration of the preceding remarks, such elevated temperatures may advantageously be achieved either by the use of heated solutions or by the use of steam, and wherein the heated solutions and steam may contain the desired hydrolyzing agents.

For a more detailed discussion of diazoimino compounds suitable for use herein reference may be had to copending application Serial No. 14,271, filed April 2, 1935, wherein these compounds are described and claimed.

By means of the present invention an entirely new class of diazoimino compounds is utilized in the production of superior dyes and prints. These compounds are quite dissimilar to any heretofore used since they are not hydrocarbon derivatives but are derivatives of heterocyclic compounds. Due to the presence of one or more hetero atoms and due to the configuration of these diazoimino compounds it is possible to produce superior colors readily and economically. The stability of these diazoimino compounds is quite marked, while at the same time the ease with which they revert to the parent diazo salt upon treatment with suitable hydrolyzing agents is most pronounced. The compounds described herein are quite compatible with assistants, penetrating agents, thickeners, alkalies, solvents and the numerous other accessories used in the production of ice color dyes and prints. The resulting colors are exceedingly uniform and level and are exceptionally fast to laundering.

As many apparently widely different embodiments of this invention may be made without departing from the spirit and scope thereof, it is to be understood that the invention is not limited to the specific embodiments thereof except as defined in the appended claims.

We claim:

1. Dyeing and printing compositions which comprise an ice color coupling component and a diazoimino compound having the following general formula:



wherein R represents the residue of a diazotized aromatic amine or tetrazotized aromatic diamine, Z represents the radical of a heterocyclic compound having an imino-containing radical substituted thereon coupling taking place through the imino group of the aforementioned substituent, said heterocyclic derivative containing at least one water-solubilizing group, and n represents the integer 1 or 2.

2. Dyeing and printing compositions which comprise an ice color coupling component and a diazoimino compound having the following general formula:



wherein R represents the residue of a diazotized aromatic amine or tetrazotized aromatic diamine of the benzene or naphthalene series, free from water-solubilizing groups, Z represents the radical of a heterocyclic compound having an imino-containing radical substituted thereon coupling taking place through the imino group of the aforementioned substituent, said heterocyclic

derivative containing at least one water-solubilizing group, and n represents the integer 1 or 2.

3. Dyeing and printing compositions which comprise an ice color coupling component and a diazoimino compound having the following general formula:



wherein R represents the residue of a diazotized aromatic amine or tetrazotized aromatic diamine, Z represents the radical of a furane derivative having an imino-containing radical substituted thereon coupling taking place through the imino group of the aforementioned substituent, said furane derivative containing at least one water-solubilizing group, and n represents the integer 1 or 2.

4. Dyeing and printing compositions which comprise an ice color coupling component and a diazoimino compound having the following general formula:



wherein R represents the residue of a diazotized aromatic amine or tetrazotized aromatic diamine of the benzene or naphthalene series, free from water-solubilizing groups, Z represents the radical of a furane derivative having an imino-containing radical substituted thereon coupling taking place through the imino group of the aforementioned substituent, said furane derivative containing at least one water-solubilizing group, and n represents the integer 1 or 2.

5. Dyeing and printing compositions which comprise an ice color coupling component and a diazoimino compound having the following general formula:



wherein R represents the residue of a diazotized amine of the benzene or naphthalene series, free from water-solubilizing groups, and Z represents a furane derivative having an imino-containing radical substituted thereon coupling taking place through the imino group of the aforementioned substituent, said furane derivative containing at least one water-solubilizing group.

6. Dyeing and printing compositions which comprise an arylamide of 2-3-hydroxy-naphthoic acid and a diazoimino compound having the following general formula:



wherein R represents the residue of a diazotized amine of the benzene or naphthalene series, free from water-solubilizing groups, and Z represents a furane derivative having an imino-containing radical substituted thereon coupling taking place through the imino group of the aforementioned substituent, said furane derivative containing at least one water-solubilizing group.

7. Dyeing and printing compositions which comprise an arylamide of 2-3-hydroxy-naphthoic acid and a diazoimino compound having the following general formula:



wherein R represents the residue of an aromatic amine of the benzene series, free from carboxylic or sulfonic acid groups.

8. Dyeing and printing compositions which comprise an arylamide of 2-3-hydroxy-naphthoic

acid and a diazoimino compound having the following general formula:



wherein R represents the residue of an aromatic 10 amine of the benzene series, free from carboxylic or sulfonic acid groups.

9. Dyeing and printing compositions which comprise an acyl-acet-arylide and a diazoimino compound having the following general formula:



wherein R represents the residue of a diazotized 20 amine of the benzene or naphthalene series, free from water-solubilizing groups, and Z represents a furane derivative having an imino-containing radical substituted thereon coupling taking place through the imino group of the aforementioned substituent, said furane derivative containing at least one water-solubilizing group.

25 10. A process for imparting color to textile fibers which comprises treating said fibers with a composition comprising an ice color coupling component and a diazoimino compound having the following general formula:



wherein R represents the residue of a diazotized 35 aromatic amine or tetrazotized aromatic diamine, Z represents the radical of a heterocyclic compound having an imino-containing radical substituted thereon coupling taking place through the imino group of the aforementioned substituent, said heterocyclic derivative containing at least one water-solubilizing group, and n represents the integer 1 or 2, and developing the treated fibers by subjecting them to the action of a hydrolyzing agent.

11. A process for imparting color to textile fibers which comprises treating said fibers with a 45 composition comprising an ice color coupling component and a diazoimino compound having the following general formula:



50 wherein R represents the residue of a diazotized aromatic amine or tetrazotized aromatic diamine of the benzene or naphthalene series, free from water-solubilizing groups, Z represents the radical of a heterocyclic compound having an imino-containing radical substituted thereon coupling taking place through the imino group of the aforementioned substituent, said heterocyclic derivative containing at least one water-solubilizing group, and n represents the integer 1 or 2, and developing the treated fibers by subjecting them to the action of a hydrolyzing agent.

12. A process for imparting color to textile fibers which comprises treating said fibers with a composition comprising an ice color coupling component and a diazoimino compound having the following general formula:



wherein R represents the residue of a diazotized 70 aromatic amine or tetrazotized aromatic diamine, Z represents the radical of a furane derivative having an imino-containing radical substituted thereon coupling taking place through the imino group of the aforementioned substituent, said furane derivative containing at least one water-

solubilizing group, and n represents the integer 1 or 2, and developing the treated fibers by subjecting them to the action of a weak acid at elevated temperatures.

13. A process for imparting color to textile 5 fibers which comprises treating said fibers with a composition comprising an ice color coupling component and a diazoimino compound having the following general formula:



wherein R represents the residue of a diazotized 15 aromatic amine or tetrazotized aromatic diamine of the benzene or naphthalene series, free from water-solubilizing groups, Z represents the radical of a furane derivative having an imino-containing radical substituted thereon coupling taking place through the imino group of the aforementioned substituent, said furane derivative containing at least one water-solubilizing group, and n represents the integer 1 or 2, and developing the treated fibers by subjecting them to the action of a weak acid at elevated temperatures.

14. A process for imparting color to textile 20 fibers which comprises treating said fibers with a composition comprising an ice color coupling component and a diazoimino compound having the following general formula:



wherein R represents the residue of a diazotized 30 aromatic amine or tetrazotized aromatic diamine, Z represents the radical of a heterocyclic compound having an imino-containing radical substituted thereon coupling taking place through the imino group of the aforementioned substituent, said heterocyclic derivative containing at least one water-solubilizing group, and developing the treated fibers by subjecting them to the action of acetic or formic acid at elevated temperatures.

15. A process for imparting color to cotton 35 fibers which comprises treating said fibers with a composition comprising an arylamide of 2-3-hydroxy-naphthoic acid and a diazoimino compound having the following general formula:



wherein R represents the residue of a diazotized 45 aromatic amine or tetrazotized aromatic diamine of the benzene or naphthalene series, free from water-solubilizing groups, Z represents the radical of a furane derivative having an imino-containing radical substituted thereon coupling taking place through the imino group of the aforementioned substituent, said furane derivative containing at least one water-solubilizing group, and developing the treated fibers by subjecting them to the action of acetic or formic acid at elevated temperatures.

16. A process for imparting color to cotton 50 fibers which comprises treating said fibers with a composition comprising an arylamide of 2-3-hydroxy-naphthoic acid and a diazoimino compound having the following general formula:



wherein R represents the residue of an aromatic 60 amine of the benzene series, free from carboxylic or sulfonic acid groups, and developing the treated fibers by subjecting them to the action 65

5

10

15

20

25

30

35

40

45

50

55

60

65

70

75

of acetic and formic acid at elevated temperatures.

17. A process for imparting color to cotton fibers which comprises treating said fibers with a composition comprising an arylamide of 2-3-hydroxy-naphthoic acid and a diazoimino compound having the following general formula:



wherein R represents the residue of an aromatic amine of the benzene series, free from carboxylic or sulfonic acid groups, and developing the treated fibers by subjecting them to the action of acetic and formic acid at elevated temperatures.

20 18. A process for imparting color to cotton fibers which comprises treating said fibers with

a composition comprising an acyl-acet-arylide and a diazoimino compound having the following general formula:



wherein R represents the residue of a diazotized amine of the benzene or naphthalene series, free from water-solubilizing groups, and Z represents a furane derivative having an imino-containing radical substituted thereon coupling taking place through the imino group of the aforementioned substituent, said furane derivative containing at least one water-solubilizing group, and developing the treated fibers by subjecting them to the action of acetic and formic acid at elevated temperatures.

MILES A. DAHLEN.  
STANLEY R. DETRICK.  
ROBERT E. ETZELMILLER.  
FRITHJOF ZWILGMEYER.